

Oct. 7, 1924.

1,511,196

J. B. AUSTIN

## PROCESS OF UNITING METALS

Filed Aug. 18, 1924



INVENTOR  
John B. Austin  
BY  
Rickey Slough & Walls  
ATTORNEYS.

## UNITED STATES PATENT OFFICE.

JOHN B. AUSTIN, OF CLEVELAND, OHIO.

## PROCESS OF UNITING METALS.

Application filed August 18, 1924. Serial No. 732,802.

*To all whom it may concern:*

Be it known that I, JOHN B. AUSTIN, a citizen of the United States, residing at 1615 Collamer Street, Cleveland, in the county of 5 Cuyahoga and State of Ohio, have invented certain new and useful Improvements in Processes of Uniting Metals, of which the following is a specification.

My invention relates to the art of uniting 10 non-ferrous to ferrous metals. More particularly it relates to a new and improved process of uniting a copper bond to the base and web of a steel railway rail. It also relates to a process of uniting copper to each 15 of two or more adjacent steel surfaces disposed at angles to each other. It further relates to a new and improved apparatus adapted to form about the copper portion of a copper bond a molten metal retaining wall 20 adapted to cooperate with a rail base and web to retain molten metal in contact with the rail base and web and with the copper of the bond while the weld is being made.

Prior to my invention it was not the practice, so far as I am aware, to unite copper bonds directly to the web of a rail by a flame without seriously weakening a portion of the web, due to the melting of a portion thereof. Although it was desirable to attach mine 25 bonds to the rail webs, because of the protection thus afforded the bond and because of the welding difficulties encountered in bonding to wet and rusty rail bases, it was considered unsafe to bond to the web of the rail 30 by any bonding process employing a heating flame because of the fear of resulting serious injury to and weakening of the rail web.

I have discovered, however, that copper 40 bonds can be directly welded to the web of a rail by means of a heating flame without any substantial melting of or noticeable injury to the rail. I have also discovered that a copper bond may be quickly and easily 45 united by means of a heating flame to both the base and web of a wet and/or rusty rail.

Briefly stated, my improved process for practicing my discoveries comprises forming a molten metal retaining wall about a 50 portion of the copper of a bond on a rail base, melting copper onto the rail base and retaining it by the said retaining wall and maintaining the copper in a molten condition until it has united with the rail base, 55 rail web and the copper of the bond. A device suitable for practicing my invention

may be described briefly as comprising a mold portion formed to cooperate with the rail base and web in providing walls to retain molten metal on the base of a rail adjacent to the rail web and thru one wall of which a portion of the copper of the bond extends.

For the purpose of disclosing my invention to those skilled in the art, I have elected 60 to describe hereinafter my new and improved process as practiced in uniting a copper bond to the base and web of a steel rail and have shown devices suitable for use in connection therewith. I do not wish to 65 be understood, however, as limiting my invention to these specific disclosures since it will be obvious to those skilled in the art that my improved process and devices may be employed in attaching copper to two or more 70 angularly disposed steel surfaces and since various modifications in the process, as well as the devices coming within the scope of my invention, will, no doubt, occur to others.

In the accompanying drawings forming a 75 part of this specification Fig. 1 is a perspective view of a rail and bond, assembled with a mold portion embodying my invention.

Fig. 2 is top plan view of the mold portion of Fig. 1.

Fig. 3 is an end elevation on line 3-3 of Fig. 2.

Fig. 4 is a side elevation on line 4-4 of Fig. 2, and

Fig. 5 is a fragmentary top plan view, 80 partly in section, of a rail and a modified form of mold portion embodying my invention.

In Figs. 1 to 4 inclusive of the drawings numeral 1 designates a fragmentary part of 85 a mine rail with a bond 2 positioned adjacent to the base and web in position to be united to the rail base and web, and 3 indicates as an entirety a device for forming with the base and web of the rail a molten 90 metal retaining mold cavity about the end 4 of the copper of the bond 2.

The device or mold portion 3 as shown in these figures seats on the rail base 1<sup>a</sup> and cooperates therewith and with the rail web 1<sup>b</sup> to retain molten metal adjacent to the end of the end 4 of the bond 2 in position to unite therewith and with the base and web of the rail. It preferably consists of a bond 105 positioning member 5, preferably composed 110 of copper, adapted to rest on the base 1<sup>a</sup>, of the rail and substantially to engage with

the web 1<sup>b</sup> of the rail, and having provided in its lower surface with a recess 6 of substantially the size and configuration of the end 4 of the bond 2 for use therewith. A 5 rib 7 acts as a stop against which a suitable flange or rib 4<sup>a</sup> on the bond may engage, thereby positioning a portion of the copper of the bond in the device 3 on the rail and preventing the escape of molten metal 10 around this part of the casting cavity thus formed. Connected to member 5 is a mold cavity forming member 8, preferably composed of carbon and likewise adapted to rest on the base of the rail and to engage with 15 the web of the rail. This member 5 is preferably cut away as at 8<sup>a</sup> to bound a portion of a mold cavity or recess 9, which is open to the recess 6 and other walls of which cavity are formed by the web and base of the 20 rail, so as to retain molten metal in contact with the rail web and base and with the copper of the bond projecting thereinto. This mold cavity is preferably open at the top so that molten metal may be brought 25 into the recess 9 through the top thereof and maintained molten therein by a heating flame directed thereinto. Other walls of the mold cavity or recess 9 are formed by the rail web and base when the mold portion 3 30 is in assembled position on to a rail base.

The members 5 and 8 may be connected together in any suitable manner. In this instance they are connected by a thin sheet metal band 10 which runs along one end and 35 one side of member 8 and one end of member 5 and carries pins 11 which project into suitable openings 11<sup>a</sup> in the member 8 and also carries a screw 12 which engages with a tapped opening 12<sup>a</sup> in member 5. A pin 13 carried by member 5 and projecting into a 40 recess 13<sup>a</sup> in the member 8 serves to position members 5 and 8 at their junction. Mold portion 3 may be held in position on a rail by any suitable means, including a clamp 45 or weight or even welding a metal part thereof to the rail.

In practicing my invention on a mine rail I first remove the mud and any other foreign material from the base of the rail, 50 without, however, taking pains to dry the rail base or remove rust, except large particles which may be knocked off readily. Then I position a bond 2 with the outstanding rib 4<sup>a</sup> contacting with the rib 7 on the member 5. The bond 2 and mold portion 3 are then 55 placed on the rail base adjacent to the rail web and retained in such position in any suitable manner. This may be done, for example, by means of a clamp or mold holder where said mold portion is detachably connected to the copper of the bond, and if it is a mold so secured to the copper bond head as to be substantially permanent therewith, that is, the mold portion is carried 60 by the bond head and is made of metal, 65

it may be welded or clamped to the rail as desired.

Copper may be melted by a suitable heating flame into the mold cavity and additional heat supplied to the copper by directing the flame on the molten copper on the rail without directing the flame on the steel and maintaining the flame thereon until the molten copper unites to a portion of the copper of the bond and to the base and web 70 of the rail. For this purpose any suitable heating flame may be used such as the electric arc or a gas flame, for example, oxy-acetylene. With the electric arc either a carbon or a metal electrode may be used. The 80 union of the copper to the rail is denoted by the wetting of the rail by the copper. This wetting action is indicated by the formation of a concave meniscus by the copper adjacent to the rail. 85

While the above process may be carried out by melting pure copper into the mold cavity, it is preferable to employ with the copper a deoxidizing agent, such as silicon in amount of about 0.25%. By employing 90 a deoxidizing agent, such as silicon, the process may be carried out in less time and probably at a lower temperature than when no deoxidizing agent is employed.

Successive increments of copper may be 95 melted into the mold cavity from the copper electrode and the arc maintained on said molten copper until sufficient copper has been melted into said mold cavity and the copper therein has united with a portion of the copper of the bond and with the base and web of the rail. The uniting of the copper to the steel will be indicated by the wetting of the steel by the copper. By employing 100 as an electrode copper having a deoxidizing agent alloyed therewith, the said agent is melted in uniform relation to the copper and is distributed uniformly throughout the bath of molten copper. By the use of said deoxidizing reagent, this process may be 105 carried out in less time and probably at a lower temperature than would be possible without the use of said reagent. It will be noted that in practicing my invention with the use of the metal arc, employing a copper electrode containing silicon, the uniting 110 of the copper to the steel is effected substantially simultaneously with the completion of the melting of the copper into the mold cavity.

It will be noted that if the rail is substantially dry and reasonably free from rust or similar substances, a clean, non-porous junction will be formed between the copper and substantially all the rail surface in contact therewith. If, however, the rail be wet or covered with a substantial coating of rust or similar substances, or both wet and covered with said substances as is often the case in the mines, the portion of the rail

base interiorly of the mold cavity may not be completely united with the copper throughout the contacting surfaces thereof, especially if the metal arc process is employed. The portion of the rail web interiorly of the mold cavity, however, will be united with the copper throughout substantially their contacting surfaces. It will be noted, however, that where the weld of the 10 copper to the steel is principally disposed along the contacting surfaces of the copper and the web portion of the rail interiorly of the mold, the area of welded contact is sufficiently large to provide sufficient mechanical strength and electrical conductivity. In the mines it is preferred to employ the metal arc in carrying out this process. In this case a copper rod may be used as an electrode. Preferably the deoxidizing 20 agent is added simultaneously with the melting of the copper and thus there may be employed a copper electrode containing about 0.25% silicon distributed substantially uniformly therein.

25 In Figure 5 I have shown a slightly different form of mold portion applied to the fragment of a rail, the sectioned part of the figure indicating the web after the head of the rail has been removed. This mold portion 15 consists of a bond positioning member 16 preferably composed of copper having a recess 17 with a rib 18 projecting therein to engage behind the rib 4<sup>a</sup> of the copper portion 4 a bond end. This member 16 is adapted to rest on the rail base 1<sup>a</sup>. At either end thereof I provide molten metal retaining wall members 19 which are preferably composed of carbon and which rest on the rail base and engage with the rail 40 web as shown.

A sheet shaped metal band 20 is bent to engage the top outer sides of members 16 and 19 and carries screws 21 which secure these members in the assembled position shown in this figure.

50 When mold portion 15 rests on a rail base and against a rail web a molten metal retaining mold cavity 22 is formed, the rail base and web constituting certain walls thereof and the members 16, 19 and the copper of a bond comprising the remaining walls thereof. The mold portion is thus open at its top to receive molten metal and to permit a heating flame to be directed onto molten metal in the mold cavity; and is open at its side and bottom to expose the rail web and base to contact with the molten metal.

55 It will be understood that under certain conditions the members 19 and 20 may be entirely omitted, retaining only the member 16 to serve as a molten metal retainer in conjunction with the rail base and web, so that the metal may be melted between this member 16 and the web of the rail in con-

tact with the rail base. The mold portion 15 shown in this figure may be used in practicing my invention in substantially the same manner as has been previously described in connection with molds shown in 70 Figs. 1 to 4.

75 It will thus be seen that my process may be carried out without injury to the rail or any deleterious effect upon the rail. As a matter of fact, a bond attached by my process does not injure the rail at the point of attachment of the bond and there is no gouging of the steel of the rail or creation of injurious effects thereon or therein by the electric arc, there being no occasion for the 80 arc to come into direct contact with the steel of the rail either on the base or on the web.

85 While I have shown and described my process as applied to the uniting of a portion of the copper of a bond to the base and web of a rail I do not wish to be understood as limiting my invention to the process specifically thereto, but I wish the scope of my invention to include the uniting of a 90 non-ferrous article to two angularly disposed surfaces of a ferrous article, and while for the sake of brevity the claims specify the word rail, I intend such word to be comprehensive of any two angularly disposed non-ferrous surfaces, and the word 95 copper in the claims to be comprehensive of any non-ferrous metal used for the purpose of conducting electricity.

100 Furthermore, it is to be understood that the particular form of apparatus shown and described, and the particular procedure set forth, are presented for purposes of explanation and illustration and that various modifications of said apparatus and procedure can be made without departing from 105 my invention as defined in the appended claims.

What I claim is:

1. The process of uniting a copper bond to a steel rail which comprises forming a 110 suitable mold cavity about a portion of the copper of a bond adjacent to a rail, of which mold cavity the base and web of the rail form mold walls, respectively, melting copper into the mold cavity, directing a heating flame on the molten copper within said cavity without directing the flame on the steel and maintaining the copper molten until the gases are substantially eliminated and the copper unites with the steel of the 120 web of the rail and the bond and forms a substantially non-porous junction between the copper and the steel.

125 2. The process of uniting a copper bond to a steel rail which comprises forming a suitable mold cavity about a portion of the copper of a bond adjacent to a rail, of which mold cavity the base and web of the rail form mold walls, respectively, melting copper from a metal arc electrode into the mold 130

- 5 cavity in the presence of a suitable deoxidizer, directing said arc on the molten copper within said cavity without directing it on the steel and maintaining the copper 45 molten until the gases are substantially eliminated and the copper unites with the steel of the web of the rail and the bond and forms a substantially non-porous junction between the copper and the steel. 50
- 10 3. The process of uniting a copper bond to a steel rail which comprises forming a suitable mold cavity about a portion of the copper of a bond adjacent to a rail, of which mold cavity the base and web of the rail 55 form mold walls, respectively, melting copper into the mold cavity, directing a heating flame on the molten copper within said cavity without directing the flame on the steel and maintaining the copper molten 60 until the copper unites with the base and web of the rail and the bond and forms a substantially non-porous junction between the copper and the steel. 65
4. The process of uniting a copper bond to a steel rail which comprises forming a suitable mold cavity about a portion of the copper of a bond adjacent to a rail, of which mold cavity the base and web of the rail 70 form mold walls, respectively, melting copper from a metal arc electrode into the mold cavity in the presence of a suitable deoxidizer, directing said arc on the molten copper within said cavity without directing it on the steel and maintaining the copper molten until the copper unites with the base and web of the rail and the bond 75 and forms a substantially non-porous junction between the copper and the steel. 80
5. The process of uniting a copper bond to a steel rail which comprises forming a suitable mold cavity about a portion of the 85
- copper of a bond of which mold cavity the base and web of the rail form mold walls respectively, melting copper into the said mold cavity into contact with the rail base and rail web, and heating the molten copper without melting a substantial amount of the rail until the copper unites with the steel of the web of the rail and with the copper of the bond. 90
6. The process of uniting a copper bond to a steel rail which comprises forming a suitable mold cavity about a portion of the copper of a bond of which mold cavity the base and web of the rail form mold walls 95 respectively, melting copper into the said mold cavity into contact with the rail base and rail web, directing a heating flame on the molten copper in the mold cavity without directing the flame on the rail, and heating the molten copper by the flame until the copper unites with the steel of the web of the rail and with the copper of the bond. 100
7. The process of uniting a copper bond to a steel rail which comprises forming a suitable mold cavity about a portion of the copper of a bond of which mold cavity the base and web of the rail form mold walls 105 respectively, melting copper into the said mold cavity into contact with the rail base and rail web, directing a heating flame on the molten copper in the mold cavity without directing the flame on the rail and without melting a substantial amount of the rail, 110 and heating the molten copper by the flame until the copper unites with the steel of the web of the rail and with the copper of the bond. 115

In testimony whereof I hereunto affix my signature this 14th day of August, 1924.

JOHN B. AUSTIN.